

## UNITED STATES PATENT OFFICE

2,150,060

## STABILIZING COLOR BINDING AGENT

Friedrich Hoermann von und zu Guttenberg, Genthin, and Rudolf Köhler, Dusseldorf-Benrath, Germany, assignors to the firm Henkel & Cie, Gesellschaft mit beschränkter Haftung, Dusseldorf, Germany

No Drawing. Original application June 15, 1935, Serial No. 26,866. Divided and this application October 25, 1937, Serial No. 170,955. In Germany June 20, 1934

2 Claims. (CL 134—50)

This invention relates to a color binding agent and more particularly to a stabilized color binding agent and to a method of stabilizing the same.

Color binding agents embodying a colloidal dispersion of an oily substance in an aqueous medium are almost always unstable structures. They are generally subject to changes of such a nature that an increase in the size of the particles of the colloidally dispersed oily substance occurs, which finally results in separation of the components. In addition, the structure of the colloidal dispersion may undergo a change in the course of time. All these processes, which are comprised in the expression "ageing phenomena" make themselves felt in an unpleasant manner in the technical application of such a color binding agent. We have now succeeded in finding an addition which stabilizes such color binding agents that are of the greatest interest for practice, and which at least represses the ageing phenomena.

According to the invention, polyphosphates are incorporated with such color binding agents. Preferably, water-soluble polyphosphates, particularly alkali polyphosphates, come into consideration. The latter may be produced by melting alkali pyrophosphates with alkali metaphosphates, or directly from their starting substances. For example, sodium polyphosphates of the formulas  $\text{Na}_5\text{P}_3\text{O}_{10}$ ,  $\text{Na}_4\text{P}_4\text{O}_{13}$ ,  $\text{Na}_11\text{P}_5\text{O}_{23}$ , and  $\text{Na}_{12}\text{P}_{10}\text{O}_{31}$  may be employed.

The use of polyphosphates for stabilizing such color binding agents is extremely varied. Color binding agents may be stabilized in which there is an extremely fine dispersion (limit region of molecular solubility) or coarser colloidal dispersion up to the limit of coarse mechanical dispersions. By the addition of polyphosphates, ageing phenomena, such as for instance flocculation, thickening of sols, gelatinisation or, in the case of jellies, syneresis, may be prevented. More particularly, concentrated colloidal dispersions, which are very subject to the said phenomena, may be stabilized by an addition of polyphosphates.

The choice of the polyphosphate depends inter alia upon the pH-value which is brought about by the polyphosphate. Preferably, polyphosphates are selected, the pH-value of which agrees with the desired optimum pH-value of the colloid.

The following are the pH-values of the polyphosphates:

|                                            | pH  | 5 |
|--------------------------------------------|-----|---|
| $\text{Na}_5\text{P}_3\text{O}_{10}$       | 8.9 |   |
| $\text{Na}_4\text{P}_4\text{O}_{13}$       | 8.3 |   |
| $\text{Na}_{12}\text{P}_{10}\text{O}_{31}$ | 7.1 |   |

The quantities of polyphosphate employed depend upon the nature of the colloidal dispersion which is to be stabilized. Frequently, the addition may be less than 1% or even less than 0.1%. The addition of polyphosphates is preferably made to technical color binding agents which are only employed some time after their manufacture. If desired, the polyphosphates may also be added to colloidal dispersions which are made or which form only immediately upon use. The polyphosphates exhibit a stabilizing effect both in the cold and when hot.

The polyphosphates may also be employed in the presence of other known stabilizing agents, such as for example decomposition products of albumen, such as lysalbinic acid. Furthermore, the soluble salts of other phosphoric acids which contain less water than orthophosphoric acid, for example alkali pyrophosphates or hypophosphates may be combined with the polyphosphates.

The polyphosphates are eminently suitable for stabilizing such color binding agents. Thus, for example, emulsions of oils in aqueous caseinate solutions are often employed for paint purposes. These emulsions may be stabilized by the addition of polyphosphates, so that even after the addition of the colour pigment, no subsequent thickening occurs, and the finished mixtures retain their good spreading properties.

## Example

A color binding agent is made by emulsifying 400 grams of linseed oil in 600 grams of a solution of 80 grams of casein in 500 grams of water and 20 grams of concentrated ammonia, with the addition of 50 cubic centimetres of a solution of 10 grams of sodium polyphosphate of the formula  $\text{Na}_5\text{P}_3\text{O}_{10}$ . If a white paint is made from 400 grams of this binding agent, 400 grams of zinc oxide and 200 grams of water, the paint retains its consistency and its good spreading powers even after long storage. Without the addition of 50

polyphosphates, subsequent thickening occurs, so that even after some time the paint becomes so stiff that it can only be spread with difficulty.

We claim.

5. 1. The method of stabilizing a color binding agent embodying a colloidal dispersion of a drying oil in an aqueous solution of an alkaline caseinate which comprises incorporating water-soluble polyphosphates therewith selected from the group consisting of Na<sub>5</sub>P<sub>3</sub>O<sub>10</sub>; Na<sub>6</sub>P<sub>4</sub>O<sub>13</sub>; Na<sub>11</sub>P<sub>9</sub>O<sub>23</sub> and Na<sub>12</sub>P<sub>10</sub>O<sub>31</sub>.

2. As a new article of manufacture, a color binding agent comprising a colloidal dispersion of a drying oil in an aqueous solution of an alkaline caseinate and stabilized by containing a predetermined quantity of a water-soluble polyphosphate selected from the group consisting of Na<sub>5</sub>P<sub>3</sub>O<sub>10</sub>; Na<sub>6</sub>P<sub>4</sub>O<sub>13</sub>; Na<sub>11</sub>P<sub>9</sub>O<sub>23</sub> and Na<sub>12</sub>P<sub>10</sub>O<sub>31</sub>. 5

FRIEDRICH HOERMANN VON  
UND ZU GUTTENBERG.

RUDOLF KÖHLER.

10